

1

3,740,345

## DYEING COMPOSITION

Wolfgang Berger, Gartenberg, Germany, assignor to Dr. Th. Bohme KG Chem. Fabrik, Gartenberg, Germany  
No Drawing. Filed Aug. 26, 1970, Ser. No. 67,202  
Claims priority, application Germany, Sept. 11, 1969,

P 19 46 058.3

Int. Cl. B01f 17/00, 17/16

U.S. Cl. 252—355

4 Claims

## ABSTRACT OF THE DISCLOSURE

Dyeing and deaerating composition including a low ethoxylated fatty acid diamine, an alkali metal salt of dinaphthyl methane disulfonic acid, and a mixture of alkali metal salts of propoxylated monoesters and diesters of phosphoric acid.

## BACKGROUND

This invention relates to a composition which is of use in the dyeing industry and is also of use as a deaerating agent. This invention also relates to a process for dyeing polyamide fibers using the said composition.

Polyamide fibers, whether in the form of woven or knitted fabrics, are difficult to dye evenly and the dyed fibers often have a streaky appearance. The causes of this streakiness are mainly physical and may be due to different degrees of stretching or drafting of the fibers and to differences in texturizing of the fibers. The streakiness is also affected to a lesser degree by the number of amino terminal groups in the polyamide fibers.

The prevention of streaky dyeing is usually unpleasant and tedious. Thus, the consumption of surface-active agents is increased, these agents being required to make dyeing even. However, the agents cause foam formation in an amount which increases with the concentration in the dye vats or baths. The foam formation is troublesome since the dye vats or baths may foam over or, with for example dyeing machines (jet machines), such a strong foaming action may occur that the process can no longer be carried out.

Many auxiliary materials have been suggested for even, streak-free dyeing or polyamide materials, for example, non-ionic and anion-active surface-active agents. The use of silicones has been proposed for eliminating foam, but the silicones lead to the formation of silicone stains which can only be removed with extreme difficulty from the material. Multi-stage processes have been proposed for eliminating the streak formation when dyeing polyamide fibers, for example by pre-boiling the material to be dyed in the presence of anion-active surface-tension agents, such as high sulfonates of fatty acid derivatives, followed by cooling in order to arrive at the required dyeing temperatures in the dyeing process proper, with addition of other surface-active agents such for example as highly ethoxylated aliphatic amines. Such processes are involved, costly and time consuming.

Increased fastness standards with dyed polyamide materials necessitate the use of dyestuffs with relatively large molecules, which result in poor migration power, thus resulting in a stronger tendency to uneven and streaky dyeing.

## SUMMARY

This invention provides a composition comprising a low ethoxylated fatty acid diamine, an alkali metal salt of dinaphthyl methane disulfonic acid, and a mixture of the alkali metal salts of propoxylated mono- and diesters of phosphoric acid.

This invention also provides a process of dyeing polyamide fibers in which the dyeing is carried out with

2

a simple preliminary boiling and without intermediate cooling in the presence of a composition comprising a low ethoxylated fatty acid diamine, an alkali metal salt of dinaphthyl methane disulfonic acid, and a mixture of the alkali metal salts of propoxylated mono- and diesters of phosphoric acid.

Preferably, the composition comprises (in percent by weight):

- 10 50% of a low ethoxylated fatty acid diamine,
- 10 30% of an alkali metal salt of dinaphthyl methane disulfonic acid, and
- 15 20% of a mixture of the alkali metal salts of propoxylated mono- and di-(2-ethylhexanol-1)-esters of orthophosphoric acid.

## DESCRIPTION

The composition may include an esterified alcohol containing 4 to 6 carbon atoms in branched or unbranched form. The low ethoxylated fatty acid diamine is preferably substantially saturated. The alkali salts may be the sodium and potassium salts.

The low ethoxylated fatty acid diamine is prepared by reacting a fatty acid diamine with a molar excess of ethylene oxide for a period of time sufficient to replace one or more hydrogens attached to nitrogen atoms with ethylene oxide groups or chains.

Dinaphthylene methane disulfonic acids have the general formula



These acids are described by Schwartz and Perry in "Surface Active Agents and Detergents," vol. I, page 119. Their alkali metal salts are prepared in the usual manner by reacting the diacid with a sodium or potassium compound such as NaOH or KOH.

Phosphoric acid mono- and diesters are prepared in the normal manner by reacting phosphoric acid with an amount of an alcohol sufficient to esterify one or two —OH groups attached to phosphorus. The mixture of mono- and diesters is then reacted with propylene oxide followed by neutralization with alkali to form a mixture of the alkali metal salts of propoxylated mono- and diesters of phosphoric acid.

The process of the invention enables streak-free, highly fast, even dyeing under technical and economic conditions. The polyamide fibers may be in woven or knitted form to give a fabric or yarn which can be evenly and streak-free dyed with a low foaming action. It is surprising that even dyeing can be obtained without special preparation of the fiber material and with a low foaming action. Moreover, shortening of the long dyeing times hitherto necessary in most cases may be obtained.

As indicated above, the composition of the invention is also suitable for use as a deaerating agent. This is because it prevents air occlusions due to its low foam and its wetting behaviour. Thus, for example, the composition may be used with texturized packages to prevent or reduce the hitherto obtained white undyed spots which are caused by air bubbles.

The advantages obtained from the present composition result from the synergistic action of the compounds present in the composition. If the compounds are used singly, then the advantages are not obtainable in the required degree. By way of example, propoxylated phosphoric acid esters, especially in normal operational 10% or more stock solutions, tend to produce flocculation. However, this flocculation does not occur when the esters are com-

bined with fatty acid diamines and sodium salts of dinaphthyl methane disulphonic acids. The ethoxylated diamines by themselves produce scarcely any effects.

Examples of the diamines which may be used are the amines of pure saturated fatty acids with chain lengths of C<sub>10</sub> to C<sub>20</sub>. Alternatively, the diamines obtained from natural or synthetic fatty acid mixtures with low iodine numbers may be used, for example the diamines produced from coconut fatty acids, palm oil fatty acids and technical stearic acids.

With dyeing temperatures above 100° C., the migrating action of the dyestuffs is considerably increased by the presence of the composition of this invention. The process of the invention can be carried out in all conventional color combinations. The advantages of the process are particularly noticeable with classes of dyestuffs which have a poor levelling action and a strong tendency to streaky dyeing, such as the phthalocyanines which are made water-soluble. Especially with "turquoise shades," strikingly better and more solid dyeings are achieved with the aid of the composition of this invention.

Dyeing is effected by initially boiling the material to be dyed for 20 to 30 minutes in the presence of up to 4% by weight of the composition, calculated on the weight of the material, and also in the presence of the other conventional chemicals required for the dyeing. This time is required when using the conventional dyeing methods in order to heat up the dye liquor from approximately 40 to 50° C. to boiling temperature. After the preliminary boiling, the dyestuff, if desired in dissolved form, is added to the bath without any addition of other auxiliary agents, and then the complete dyeing is carried out for one hour by boiling or at high temperatures. The material is completely dyed without requiring more time and increased expense, and satisfactory, level, streak-free dyeing is obtained also when using true dyestuffs.

The composition of the invention can, in general, be used in amounts of approximately 3-4% by weight based on the weight of the material. In contrast, total quantities of anion-active and non-ionic auxiliary agents of 6-10% are necessary according to the known methods. In the known methods, this has the result that, for example with polyamide material which would be roughened after the dyeing, the material can only be inadequately roughened or not satisfactorily roughened because of the high quantities of added auxiliary agents. It is believed that the cohesive components contained in the roughening and brightening agents become ineffective because of the larger quantities of previously introduced auxiliary agents. These disadvantageous effects may be avoided when using the composition of the present invention.

The invention will now be illustrated with reference to the following examples which are not intended to limit the invention in any manner. All percentages are by weight unless indicated otherwise.

**Example 1**—Good dyeing of polyamide materials which tends to dye with a streaky effect by using a composition according to the invention

The polyamide material was pretreated by boiling for 20 minutes with 2% of the composition described below and 2% of 60% acetic acid. Thereafter, 1.5% of Acid Blue (C.I. 26360) was added at boiling temperature and dyeing took place for 60 minutes at 100° to 110° C.

Using this working method, level and solid dyeing effects were obtained with only a single dye auxiliary. Best possible covering of the affinity differences of the fibers (streakiness) caused by the polyamide material was obtained and the working procedure was economical.

In addition, the known strongly migrating dyeing auxiliaries cause a fairly strong, undesirable foam development in the circulating treatment baths and as a consequence it is necessary to incorporate additional defoaming products. It is an additional advantage of the invention that dyeing can be effected in conditions which are

almost free from foam, even with strong liquor circulation, therefore additional supplies of defoaming agents are unnecessary.

The composition used in this example was as follows:

- 5 (1) 50 parts by weight of low ethoxylated stearic fatty acid propylene diamine prepared by reacting stearic fatty acid propylene diamine with 15 moles of ethylene oxide (EtO) according to the following equation:



wherein x+y+z=15.

- (2) 30 parts by weight of the sodium salt of dinaphthyl methane disulfonic acid.  
 (3) 20 parts by weight of the sodium salts of propoxylated mono- and di-(2-ethylhexanol-1)-esters of orthophosphoric acid prepared by reacting 0.124 mol orthophosphoric acid with 0.372 mol 2-ethylhexanol-1 which results in a mixture containing about 60% of the monoester and about 40% of the diester according to Hochwalt et al., Ind. Eng. Chem., 34, 20 (1942), Stewart and Crandall, Am. Chem. Soc. J., 73, 1377 (1951), and U.S. Pat. No. 2,658,909. The mixture, which has an acid number of 292 mg. KOH/g. substance, is reacted with 0.38 mol propylene oxide forming a propoxylated mixture having an acid number of 183. The remaining acid is then neutralized with alkali to form the sodium salt. It is not known if propylene oxide reacts preferably with the —OH groups in the monoester or the diester but in any event, free acid remains at the end of the reaction which is neutralized to form the alkali metal salt.

The added quantity of auxiliaries was calculated on the basis of a 100% product. Where the concentration is chosen to be lower on practical grounds, the added quantity of auxiliary agents is obviously increased accordingly, for example from 2% to 4% for a 50% product.

**Control I.**—Known dyeing of polyamide material which tends to dye with streaky effect by using two dyeing auxiliary agents and a two-stage working procedure.

The material was pretreated by boiling for 20 to 30 minutes with 2% of an auxiliary agent based on highly sulphonated oleic acid and 2% of 60% acetic acid (pH 5). Thereafter, 2% of a relatively highly ethoxylated stearic fatty acid diamine was added to this bath and then circulated for 10 to 15 minutes. 1.5% of Acid Blue 113 (C.I. 26360) was thereafter added to the bath at boiling temperature and dyeing was carried out for 60 minutes at 100° or 110° C.

Despite the use of two dyeing auxiliary agents, the evenness of the dyeing was not as good as that obtained in Example 1, and the dyeing procedure in Example 2 as longer than in Example 1.

**Control II.**—Known dyeing of polyamide material by using a known customary working method and one dyeing auxiliary agent, the one dyeing auxiliary agent giving a sufficient levelling action but non-removal of the streakiness caused by the material.

The material was pretreated at 40° C. in a bath containing 2% of an auxiliary agent based only on ethoxylated stearic fatty acid diamines or such diamines in admixture with anion-active components which have an affinity for the fiber, such for example as alkyl-aryl sulphonates, mersolates, and sulphonated oleic acids, and 2% of 60% acetic acid. After 10 minutes, 1.5% of Acid Blue (C.I. 26360) was added. This dye bath was brought from 40° C. to boiling point in 30 to 45 minutes and dyeing took place at boiling point for 60 minutes.

Using such an auxiliary agent, a fully level dyeing can be obtained on the basis of a sufficient dyestuff migration action. However, such products by themselves are ineffective when using this working method for removing the streakiness caused by the material.

What is claimed is:

1. Composition consisting essentially of a ethoxylated fatty acid diamine derived from a fatty acid having a chain length of  $C_{10}$  to  $C_{20}$  prepared by reacting a fatty acid diamine with a molar excess of ethylene oxide for a period of time sufficient to replace at least one hydrogen attached to a nitrogen atom with an ethylene oxide group, an alkali metal salt of dinaphthyl methane disulphonic acid, and a mixture of alkali metal salts of propoxylated mono- and di-(2-ethyl hexanol-1) esters of orthophosphoric acid, said composition comprising 50% of said ethoxylated fatty acid diamine, 30% of said alkali metal salt of dinaphthyl methane disulphonic acid, and 20% of said mixture of alkali metal salts of propoxylated mono- and di-(2-ethyl hexanol-1) esters of orthophosphoric acid.
2. Composition of claim 1 wherein said ethoxylated fatty acid diamine is substantially saturated.

3. Composition of claim 1 wherein said ethoxylated fatty acid diamine is derived from a natural or synthetic fatty acid with a low iodine number.

4. Composition of claim 3 wherein the fatty acid is selected from the group of coconut fatty acid, palm oil fatty acid and stearic acid.

#### References Cited

##### UNITED STATES PATENTS

10 2,658,909 11/1953 Crandall ----- 260—990

##### OTHER REFERENCES

Schönenfeldt, Surface Ethylene Oxide Adducts, Pergamon Press, pp. 97 & 99 (1970).

15 Schwartz & Perry, Surface Active Agents & Detergents, vol. I, p. 119 (1949).

JOHN D. WELSH, Primary Examiner

U.S. Cl. X.R.

20 252—8.75; 8—171; 252—8.9